

Jan. 3, 1939.

F. R. HENSEL ET AL

2,142,671

COPPER ALLOY

Filed Nov. 9, 1936

HARDNESS VS. AGEING TIME  
CONDUCTIVITY VS. AGEING TIME



INVENTORS

Franz R. Hensel  
BY Earl I. Larsen  
Lundström

ATTORNEY

## UNITED STATES PATENT OFFICE

2,142,671

## COPPER ALLOY

Franz R. Hensel and Earl I. Larsen, Indianapolis, Ind., assignors to P. R. Mallory & Co., Inc., Indianapolis, Ind., a corporation of Delaware

Application November 9, 1936, Serial No. 109,822

## 1 Claim. (Cl. 219—4)

This invention relates to alloys and more particularly to copper base alloys of improved characteristics, the present application comprising a continuation in part of our copending application, Serial No. 90,865, filed July 16, 1936, since matured into Patent No. 2,123,629, dated July 12, 1938.

An object of the invention is to produce an improved copper base alloy.

10 A further object is to provide an alloy, the physical properties of which can be improved by heat treatment.

An additional object of the invention is to improve the hardness and other characteristics of 15 a precipitation hardened copper alloy.

Other objects of the invention will be apparent from the following description taken in connection with the appended claim.

The present invention comprises the combination of elements, methods of manufacture, and the product thereof brought out and exemplified in the disclosure hereinafter set forth, the scope of the invention being indicated in the appended claim.

25 While a preferred embodiment of the invention is described herein, it is contemplated that considerable variation may be made in the method of procedure and the combination of elements without departing from the spirit of the invention.

The invention may be better understood from the following description when read in conjunction with the accompanying drawing in which:

30 The figure is a graph illustrating the improvement in hardness and conductivity obtained during the age hardening of an alloy made according to the present invention.

The present invention relates to an improved copper base alloy containing cobalt, phosphorus and beryllium. It has been found that by adding cobalt and phosphorus to copper an intermetallic compound of cobalt phosphide can be formed which has a variable solid solubility in the copper matrix. We have discovered that the addition of beryllium improves these alloys, the improvement in hardness and electrical conductivity obtained by the additions of beryllium being accentuated by a suitable age hardening process.

50 The alloy may be produced as follows:

Copper is melted under glass or charcoal slag and superheated. A hardener containing 75% cobalt and 25% copper is added as a convenient means to incorporate cobalt. The beryllium may be similarly added. Phosphorus is then added in

the form of phosphor copper or some other suitable means.

In the molten condition, the alloy is extremely fluid and pours very easily.

The proportions of cobalt and phosphorus may each be varied over a considerable range of values and there may be an excess of either in some instances without deleterious effects on the alloy. The preferred weight ratio of phosphorus to cobalt is approximately 1 to 6. However, considerable age-hardening is obtained with the ratio 1 to 3 and also with a ratio as high as 1 to 10.

A slight excess of phosphorus above the amount required to form certain intermetallic compounds of cobalt phosphide will ordinarily serve as a de-oxidizing agent during the production of the alloy.

The cobalt phosphide is suitable as an age hardening ingredient for copper or certain copper alloys. The beryllium produces additional bene- 20

25

Where the cobalt, phosphorus and beryllium are added to copper the ingredients may be present in the following ranges of proportions:

|            | Per cent  | 25 |
|------------|-----------|----|
| Cobalt     | 0.05 to 5 |    |
| Phosphorus | 0.01 to 2 |    |
| Beryllium  | 0.01 to 2 |    |
| Copper     | Balance   | 30 |

The preferred proportions, however, are substantially as follows:

|            | Per cent    | 35 |
|------------|-------------|----|
| Cobalt     | 2 to 3      |    |
| Phosphorus | 0.2 to 0.75 |    |
| Beryllium  | 0.01 to 0.5 |    |
| Copper     | Balance     |    |

After the alloy has been produced it may be heated to a relatively high temperature above 700° C. and preferably in the order of 800° C. to 40 1000° C. and then rapidly cooled from that temperature to room temperature or below, preferably by quenching in water. After the quenching operation the alloy, in such form as may be desired, may be given an aging treatment by baking 45 at a temperature below 700° C. and preferably at a temperature in the order of 350° C. to 650° C. The aging may proceed for a considerable length of time according to the temperature used. The most rapid improvement in hardness and electrical conductivity will be obtained during the first two or three hours if 450° C. is used as aging temperature but further improvement will be obtained upon continuing the aging for 8 to 16 50 hours or more.

55

The improvement in hardness and electrical conductivity during aging is shown in the graphs of the figure for a representative alloy made according to the present invention in comparison with an alloy of similar composition except for the absence of beryllium. The representative alloy has the following composition:

|               | Per cent |
|---------------|----------|
| Cobalt        | 2.37     |
| 10 Phosphorus | 0.63     |
| Beryllium     | 0.3      |
| Copper        | Balance  |

The proportions of ingredients in the comparison alloy are the same with the exception that 15 beryllium is absent.

In the figure, curve 1 represents the increase in Rockwell B hardness of specimens of the comparison alloy in which no beryllium is present, quenched from 950° C. in water and aged at 450° 20 C. in air. It will be noted that that hardness was increased from about 26 Rockwell B immediately after quenching to about 62 Rockwell B after aging for 8 or more hours at 450° C. Curve 2 represents the increase in hardness of the 25 representative alloy given above containing 0.3% beryllium. It will be noted that the hardness of the beryllium-containing alloy while initially less eventually reaches a higher value than the hardness of the alloy without beryllium. The hardness 30 of the beryllium-containing alloy increases from about 24 Rockwell B immediately after quenching to about 68 Rockwell B after aging for about 16 hours.

Curve 3 in the figure represents the improvement 35 in electrical conductivity of the comparison alloy during the age hardening treatment. It will be noted that the conductivity increased from about 27% of that of copper after quenching to 55 or 56% after aging for 4 or more hours. 40 Curve 4 represents the increase in conductivity of the alloy containing 0.3% beryllium. It will be noted that the conductivity of the beryllium-containing alloy is somewhat greater regardless of the aging time, the conductivity increasing 45 from about 35% of that of copper after quenching to above 60% after aging for 4 hours or somewhat longer.

While the comparison alloy containing no beryllium exhibited little change in hardness or 50 conductivity after 4 to 8 hours aging the beryllium-containing alloy increased considerably in hardness upon further aging, the maximum being reached after aging for more than 16 hours.

By varying the proportions of the ingredients 55 in the alloy, it is possible to obtain even higher electrical conductivity and hardnesses.

After the aging treatment the material may be cold worked by rolling, for example. The hardness will be increased by cold working while the 60 electrical conductivity is not materially changed thereby.

The alloy of the present invention is able to withstand high temperatures without losing its hardness or high conductivity. The hardness 65 and conductivity of the age-hardened alloy may be maintained at temperatures considerably above the aging temperatures used and that of the cold worked alloy may also be maintained at relatively high temperatures such as at 400° C. 70 or greater.

The present alloy is easy to produce. In pouring the alloy it shows a clean stream and great fluidity.

No difficulty due to cracking or checking is encountered in hot rolling and cold working of 5 this alloy.

In the binary copper-cobalt system the solubility of cobalt in copper decreases with decreasing temperature, the cobalt being soluble in copper in the solid state only to a very limited extent. At 1000° C. 3.5% cobalt is held in solid solution by copper. At 600° C. only 0.9% cobalt is held in solid solution and at room temperature this percentage decreases to approximately 0.35%.

By adding phosphorus, cobalt phosphide is formed and this compound has a lower solid solubility in copper than does cobalt. The precipitation hardening effect is therefore greater. In age-hardened alloys the hardening ingredients 20 greatly decrease the electrical conductivity to the extent in which they are held in solid solution. Cobalt phosphide, therefore, produces a higher electrical conductivity for the same amount of hardening than does straight cobalt since less of 25 the phosphide is held in solid solution.

Another advantage accrues from the fact that the precipitated phase, consisting of cobalt phosphide or copper cobalt phosphide has in itself a substantial hardness. The hardness of this 30 phase is much greater than the precipitated phase in binary copper-cobalt alloys. This makes for greater strength and higher hardness in the hardened alloy.

The alloy is particularly suitable for pressure 35 exerting welding electrodes such as spot welding electrodes because of its combination of high hardness and electrical conductivity. This results in greater freedom from mushrooming in service. The electrodes are well adapted for the 40 welding of terne and tin plate.

The alloy also makes excellent soldering iron 45 tips due to its freedom from intercrystalline penetration of liquid metals. We have found it superior in this respect to most of the present 50 copper base alloys.

The alloy is likewise well adapted to other applications where the combination of relatively high electrical conductivity combined with high strength and hardness at room or elevated 55 temperatures is required.

It is apparent from the curves of the drawing that the beryllium makes possible alloys of considerably greater hardness and surprisingly, the 55 beryllium also appears to improve the electrical conductivity.

While the present invention, as to its objects and advantages, has been described herein as carried out in specific embodiments thereof, it is not desired to be limited thereby but it is 60 intended to cover the invention broadly within the spirit and scope of the appended claim.

What is claimed is:

An electrical contacting element of the type comprising pressure exerting welding electrodes 65 and the like composed of an alloy containing about .05 to 5% cobalt, .01 to 2% phosphorus, .01 to 2% beryllium and the remainder substantially all copper.

FRANZ R. HENSEL.  
EARL I. LARSEN.

70